

# UNITED STATES PATENT OFFICE.

ROBERT A. HADFIELD, OF SHEFFIELD, ENGLAND.

## PROCESS OF MAKING ALLOYS.

1,061,373.

Specification of Letters Patent.

Patented May 13, 1913.

No Drawing.

Application filed July 5, 1908. Serial No. 324,895.

*To all whom it may concern:*

Be it known that I, ROBERT ABBOTT HADFIELD, a subject of the King of Great Britain, of Sheffield, England, have invented a 5 certain new and useful Improvement in Processes of Making Alloys, of which the following is a specification.

In U. S. Letter Patent No. 745,829 granted to me December 1, 1908, I have set forth an 10 alloy of iron with silicon, or other material magnetically equivalent to silicon in the mixture, which is subjected to a described heat treatment; whereby a magnetic material is produced possessing magnetic permeability 15 and electric resistance above, and hysteresis quality below, those respectively of the best Swedish charcoal iron (or generally of the purest iron commercially obtainable), and hence especially adapted for use in ballast 20 coils, transformer plates and like electrical apparatus wherein the reduction of the total magnetic and electric losses to the lowest possible degree is of great importance.

My present invention is a process of making 25 alloys and more particularly such an alloy as described in the foregoing paragraph, whereby improved solidity and homogeneity of structure is obtained.

The best mode I now know of carrying 30 my said process into effect is as follows:— I place in any suitable ladle or other vessel, ferro-silicon containing preferably 50 per cent. of silicon, and raise the same to red-heat. In another vessel, I melt pure iron. 35 I pour the molten iron upon the red-hot ferro-silicon, thereby producing fusion of the same. The resulting mixture is cast in ingots in the usual way. Just before casting I preferably add a suitable proportion 40 of aluminium, or other equivalent dioxider.

The important feature of my before described process is the preliminary heating of the ferro-silicon. Inasmuch as this substance fuses at a temperature about 300° to 45 400° centigrade below that of molten iron, it is obvious that the disparity of temperature between red-hot ferro-silicon and molten iron is so small that the additional 50 heat units necessary to bring the ferro-sili-

con to fluidity are readily communicated to it from the iron itself. It is therefore not necessary to raise the iron to a temperature sufficiently high to fuse cold ferro-silicon, which might result in boiling of the iron 55 and consequent impairment of the physical properties of the resulting alloy. A still further advantage depends upon the fact that the specific gravity of the ferro-silicon is about one quarter less than that of the 60 iron—so that the ferro-silicon rises through the fluid iron poured upon it and disseminates itself through the mass much more rapidly and effectively than if it were added to the molten iron upon the surface of which 65 it would float. The iron-silicon alloy thus produced has, as has been stated, superior physical qualities in solidity and homogeneity, but these may be still further improved by the addition of aluminium in proportion not exceeding one per cent, just before the pouring of the mixture takes place. The aluminium then acts promptly upon such gases as may remain occluded in the 70 molten mass and before the latter has opportunity to absorb impurities which it might 75 not successfully attack.

I claim:

The herein described process of producing a ferro-silicon alloy for magnetic purposes, characterized by its low hysteresis and high magnetic permeability and electric resistance which consists in placing in the ladle ferro-silicon containing about 50% of silicon, raising the ferro-silicon to a red heat, 80 melting pure iron in another vessel, pouring the molten iron over the ferro-silicon so that the ferro-silicon is easily melted and disseminates itself through the mass rapidly and effectively and then adding, just before 85 the pouring of the mixture takes place, aluminium in a proportion not exceeding 1%, then casting into ingots.

In testimony whereof I have signed my name hereto in the presence of two witnesses. 95

ROBERT A. HADFIELD.

Witnesses:

HENRY E. DIXON,  
FRANK HUTSON.